

# UNITED STATES PATENT OFFICE.

PAUL H. CRAWFORD, OF DIVISADERO, SALVADOR.

## BELT-DRESSING.

1,242,424.

Specification of Letters Patent.

Patented Oct. 9, 1917.

No Drawing.

Application filed September 1, 1915. Serial No. 48,461.

To all whom it may concern:

Be it known that I, PAUL H. CRAWFORD, a citizen of the United States, residing at Divisadero, Salvador, Central America, have 5 invented new and useful Improvements in Belt-Dressings, of which the following is a specification.

This invention relates to a new and useful composition of matter for use as a belt 10 dressing, and pertains especially to a dressing which, when applied to a belt, will form a metallic wearing surface of great durability.

My composition consists of the following 15 ingredients, combined in about the proportion stated, viz:

|                       |               |         |
|-----------------------|---------------|---------|
| Linseed oil           | approximately | 9 lbs.  |
| Rosin                 | "             | 1 lb.   |
| 20      Aluminum dust | "             | 10 lbs. |

These ingredients are mixed by heating the linseed oil and rosin to form a liquid. The aluminum dust is then added and 25 thoroughly mingled by agitation until a paste is formed.

The metallic belt dressing is applied to the surface of belts and pulleys and forms 30 a coating thereon which protects the belt from marring. It also reduces loss by friction and increases the life of the belt, as the dressing has a tendency to dry and harden to a certain extent, thus forming a metal wearing surface on the inner side of the 35 belt.

In regard to this preparation, the essen-

tial feature is the metallic dust which gives the belt the metallic wearing surface. It lengthens the life of both old and new belts. The rosin and linseed oil are in the nature 40 of carriers or vehicles for the metallic dust. With the different carriers the above proportions may be varied more or less, but the formula given is one that is shown to work satisfactorily in practice.

Having thus described my invention, what 45 I claim and desire to secure by Letters Patent is:—

1. A metallic belt dressing consisting of linseed oil, rosin and aluminum ground to 50 a high state of fineness combined in about the proportions described.

2. The herein described composition of matter to be used as a belt dressing consisting of nine pounds of linseed oil, one pound 55 of rosin and ten pounds of aluminum ground to a high state of fineness.

3. A metallic belt dressing consisting of a metal ground to a high state of fineness, oil and rosin combined and used substantially in the proportions described.

4. A belt dressing consisting of oil, rosin and a finely ground metallic substance used and combined approximately in the proportions described.

In testimony whereof I have hereunto set my hand in the presence of two subscribing witnesses.

PAUL H. CRAWFORD.

Witnesses:

W. W. HEALEY,  
M. E. EWING.